# EUROPEAN PATENT SPECIFICATION

(11) **EP 3 124 650 B1**
(45) Date of publication and mention of the grant of the patent: **10.04.2019**
(21) Application number: 14886931.6
(22) Date of filing: 08.09.2014
(51) Int. Cl.: C23F 1/28, B24C 1/06, C21D 7/06, C23F 1/00, F28F 1/12, F28F 21/08

(54) **METHOD FOR PROCESSING SURFACE OF STAINLESS STEEL, AND HEAT EXCHANGER OBTAINED USING SAME**
OBERFLÄCHENBEHANDLUNGSVERFAHREN VON ROSTFREIEM STAHL UND DAMIT HERGESTELLTER WÄRMETAUSCHER
PROCÉDÉ POUR LE TRAITEMENT DE SURFACE D'ACIER INOXYDABLE ET ÉCHANGEUR DE CHALEUR OBTENU EN L'UTILISANT

(30) Priority: 25.03.2014 JP 2014061118
(43) Date of publication of application: 01.02.2017
(73) Proprietor: Hitachi, Ltd., Chiyoda-ku Tokyo 100-8280 (JP)
(72) Inventor: KAWAMURA Toshinori, Tokyo 100-8280 (JP); TAMURA Akinori, Tokyo 100-8280 (JP); NAKANO Hiroshi, Tokyo 100-8280 (JP); KITO Kazuaki, Tokyo 100-8280 (JP)
(74) Representative: Manitz Finsterwald Patent- und Rechtsanwaltspartnerschaft mbB
(86) International application number: PCT/JP2014/073606
(87) International publication number: WO 2015/145808

(56) References cited:
- WO-A2-2006/001818
- CN-A- 102 260 775
- DE-A1- 2 653 394
- JP-A- H08 218 151
- JP-A- S55 122 872
- JP-A- 2002 053 936
- JP-A- 2009 068 079

## Description

### Technical Field

The present invention relates to a surface treatment method for stainless steel. A surface treatment method as described in the preamble portion of patent claim 1 has been known from WO 2006/001818 A2.

### Background Art

Stainless steels are excellent in strength and corrosion resistance and hence, are used in a variety of applications including architectural members, hygienic members and materials for electric appliances and the like. In recent years, a stainless steel further increased in the corrosion resistance by laminating a coating material or resin film on its surface has been often used. When laminating the stainless steel with the coating material or resin film, the surface of stainless steel must be roughened for enhancing adhesion between the stainless steel and the coating material or resin film. Surface roughening techniques for stainless steel include: blasting for physically forming an irregular surface; roughening etching for chemically or electrically forming the irregular surface; and combinations thereof. For example, JP 2001-11662 A proposes a method for chemically and uniformly roughening the surface of stainless steel by using an etching solution based on sulfuric acid, chlorine ions and cupric ions. Further, JPH 5-264045 A proposes a method where sandblasting is followed by chemical etching with hydrofluoric acid, nitric acid, hydrochloric acid or aqueous solution of phosphoric acid.

WO 2006/001818 A2 discloses a stainless-steel surface treatment method for forming a fine structure on a surface of stainless steel comprising: a first step of performing grain refining treatment for refining crystal grains in the surface of stainless steel; and a second step performed, after the first step, for roughening etching the surface of stainless steel with an etching solution.

### Summary of Invention

### Technical Problem

According to the surface roughening technique using the etching treatment disclosed in JP 2001-11662 A and the like, an irregular structure is formed by preferentially etching crystal grain boundaries. Therefore, the dimensions such as width and height of the irregular structure depend upon the crystal grain size of stainless steel. It is almost impossible to form the irregular structure in dimensions of 10 µm or less because general stainless steel has the crystal grain sizes in the range of 10 to 200 µm. Although it is possible to reduce the height of projections by reducing the etching amount, the structure is reduced in surface area with the decrease in height. In a case where a fine structure having a height of 5 µm is formed by the surface roughening technique using the etching treatment, the structure achieves in maximum a surface area of about 14 times the area of a smooth surface. It is impossible to further increase the surface area of the fine structure.

According to JPH 5-264045 A, the combination of sandblasting and etching treatment provides the formation of a complicated irregular structure. However, a major irregular structure constituting a base is formed by sandblasting using abrasive grains having particle sizes on the order of 100 µm. It is therefore almost impossible to form the irregular structure in a dimension of 10 µm or less.

In this connection, an object of the present invention is to provide a stainless-steel surface treatment method for forming a fine irregular structure (roughened surface) having a high surface area on the surface of stainless steel.

### Solution to Problem

According to the present invention the above problem is solved by a stainless-steel surface treatment method having the features of, a stainless steel material according to claim 7 and a heat exchanger using the same as described in claim 8.

### Advantageous Effects of Invention

The present invention can provide a stainless-steel surface treatment method by which a fine irregular structure (roughened surface) having a high surface area can be formed on the stainless steel.

### Brief Description of Drawings

Fig. 1 is a schematic flow chart showing a process of forming a surface fine-structure.
Fig. 2 is a group of sectional views of a substrate undergoing the process of forming the surface fine-structure.
Fig. 3 shows SEM images of surfaces and cross-sections of surface fine-structures, and surface area ratios thereof.
Fig. 4 shows the results of cross-sectional crystal observation after grain refining treatment.
Fig. 5 shows the results of passive film evaluation before and after the formation of surface fine-structure.
Fig. 6 shows the results of corrosion resistance evaluation before and after the formation of surface fine-structure.
Fig. 7 is a structure diagram of a shell and tube heat exchanger according to a second embodiment of the present invention. Description of Embodiments

The embodiments of the present invention will hereinbelow be described with reference to the accompanying drawings.

Fig. 1 is a flow chart showing the steps of a process of forming a surface fine-structure of stainless steel according to the present invention.

As shown in Fig. 1, the process of the present invention is carried out in the order of grain refining treatment (first step) and roughening etching treatment (second step). It is noted that displacement deposition metal removing treatment (third step) is performed after the roughening etching treatment (second step).

A stainless-steel surface treatment method of the present invention for forming a fine structure on the surface of stainless steel is featured by refining crystal grains in the surface of stainless steel, followed by preferentially etching grain boundaries. Provided that R1 denotes an irregular structure formed by grain refining treatment of a first step, R2 denotes an irregular structure formed by roughening etching treatment as a second step, and R3 denotes an irregular structure formed by displacement deposition metal removing treatment as a third step, as shown in Fig. 2, a final surface fine-structure obtained according to the present invention is R2 or R3. That is, the surface fine-structure obtained according to the present invention does not include the irregular structure (R1) formed by the grain refining treatment of the first step. While the sizes of the irregular structures are arranged in ascending order R3<R2«R1, the sizes of R2 and R3 are substantially the same, suggesting that sufficiently fine irregular structures can be formed. These features assure that a fine roughened surface having a high surface area can be formed on the stainless steel.

The grain refining treatment (first step) is processing for forming a fine crystal layer in the surface by refining crystal grains in the surface of stainless steel. This fine crystal layer has a thickness of 1 µm or more and grain sizes of 1 µm or less because the final surface fine-structure formed according to the present invention is highly dependent on the thickness and the grain sizes of the fine crystal layer formed by this grain refining treatment. It is noted that the general stainless steel has grain sizes of 10 µm or more. The grain refining treatment method is one of either a peening treatment, grinding, turning, machining with grinder, and the like. Above all, the peening treatment is preferred which is adapted for adjustment of the thickness and grain size of the fine crystal layer according to machining conditions such as abrasive grain size and pressure.

The roughening etching treatment (second step) is processing for preferentially etching the crystal grain boundaries of the fine crystal layer formed by the first step. Therefore, the composition of a roughening etching solution has strong acidity and contains chloride ions and transition metal ions capable of displacement deposition on iron. The chloride irons have an effect to destroy a passive film composed mainly of chromium oxide generated on the stainless steel surface. The chloride ions are not particularly limited. Examples of the usable chloride irons include hydrogen chloride, sodium chloride, potassium chloride, and the like. The transition metal ions capable of displacement deposition on iron have an effect to accelerate the etching of the crystal grain boundaries by inducing the displacement deposition of a metal on iron as a main component of the stainless steel so as to suppress the etching of stainless steel. Preferred transition metal ions capable of displacement deposition on iron are those having an electric potential nobler than a standard potential of iron -0.44(V) and providing high potential difference, which include copper (+0.34(V)), silver (+0.80(V)), palladium (+0.99(V)), platinum (+1.19(V)), and gold (+1.50(V)). Particularly preferred are copper ions which are less costly.

The displacement deposition metal removing treatment (third step) is processing for preferentially etching the metal deposited on the stainless steel surface in the second step. Non-selective etching treatment is less preferable because the surface fine-structure constituting the stainless steel is etched away together with the deposited metal. It is therefore important that the composition of the solution used for the displacement deposition metal removing treatment does not contain chloride ions or nitrate ions that accelerate the etching of stainless steel and has a high dissolution rate ratio for stainless steel. It is noted that the solution composition varies depending upon the type of displacement deposition metal. In a case where the displacement deposition metal is copper, a solution composition containing persulfate or hydrogen peroxide is preferred. In a case where the displacement deposition metal is gold, platinum, palladium, or silver, a solution composition containing potassium cyanide or ammonium peroxosulfate is preferred.

The third step is performed in a case where the presence of the displacement deposition metal adversely affects the fine structure on the stainless steel surface in terms of product characteristics. In a case where the surface fine-structure is required of corrosion resistance, for example, it is preferred to perform the displacement deposition metal removing treatment if the displacement deposition metal is copper which is prone to oxidation.

### (Surface/Cross-section Observation Method)

A scanning electron microscope (SEM) was used for surficial and cross-sectional observation of the surface fine-structure. The height and width of the surface fine-structure were determined from cross-sectional SEM images. In this test, out of projections shown in the cross-sectional SEM image, five projections having greater heights and widths were measured. The measured values were averaged out and the average values were identified as the height and width of the projection of the surface fine-structure.

### (Surface Area Evaluation Method)

Krypton gas adsorption method was used for measuring the surface area. The measured surface area was evaluated in terms of surface area ratio on the basis of a smooth test piece not subjected to the process of forming the surface fine-structure.

### (Passive Film Evaluation Method)

For passive film evaluation, surface chromium concentration was measured by Auger electron spectroscopy analysis method. The measured surface chromium concentration was evaluated in terms of surface chromium concentration ratio on the basis of the smooth test piece not subjected to the process of forming the surface fine-structure.

### (Fine Crystal Layer Observation Method)

Electron Backscatter Diffraction method (EBSD) was used for observation of the fine crystal layer. OIM-Analysis commercially available from TSL Solutions Ltd. was used as a crystal orientation analysis software.

### (Corrosion Resistance Evaluation Method)

A combined cycle test complying with "Neutral Salt Spray Cycle Test Method" JISK5600-7-9 was performed for evaluation of corrosion resistance. The number of test cycles was 42. The corrosion state was evaluated according to the rating number method JISZ2371 Appendix 1 (Specifications).

### (Adhesion Evaluation Method)

An adhesion evaluation test was performed as follows. Polyimide (Hitachi Chemical Co., Ltd.) was applied to test pieces in a thickness of 50 µm and the polyimide film was peeled off with an adhesive tape.

### First Embodiment

A first embodiment is described by way of an example where wet peening treatment was used as the grain refining treatment (first step); a roughening etching solution containing copper ions as the transition metal ions capable of displacement deposition on iron was used in the roughening etching treatment (second step); and a displacement deposition metal removing solution containing persulfate was used in the displacement deposition metal removing treatment (third step). The test pieces were made of SUS304.

### (1) Grain Refining Treatment (First Step)

The wet peening treatment used glass pellets having a diameter of about 50 µm as abrasive grains and was performed under the conditions: air pressure of 0.33 MPa and conveyance speed of 20 mm/sec. It is preferred to adjust the wet peening treatment conditions according to a required crystal grain size and a required thickness of the fine crystal layer.

### (2) Roughening Etching Treatment (Second Step)

The composition of the roughening etching solution included: 500 g/l of sulfuric acid; 90 g/l of sodium chloride; and 30 g/l of cupric chloride dehydrate. The treatment was performed at a solution temperature of 40 °C for treatment time of 5 min. The treatment time may preferably be adjusted according to the etching amount required.

### (3) Displacement Deposition Metal Removing Treatment (Third step)

The composition of the displacement deposition metal removing solution included: 200 g/l of sodium persulfate; and 50 ml/l of sulfuric acid which are capable of selective removal of copper, because the roughening etching solution of the second step employed copper as the transition metal ions capable of displacement deposition on iron. The treatment was performed at a solution temperature of 30 °C for treatment time of 10 min. The treatment time may preferably be adjusted according to the amount of deposited metal.

The test pieces of the first embodiment were subjected to the surficial and cross-sectional observation by SEM, the surface area evaluation and the fine crystal layer observation.

Fig. 3 shows the results of the surficial and cross-sectional observation by SEM and the surface area evaluation. It is confirmed from the surficial and cross-sectional SEM images shown in Fig. 3 that the fine structure having a width of 1 µm or less and a height of about 3 µm is formed. The surface area of this fine structure was 21 times the area of the smooth surface. This indicates that the surface fine-structure having a height of 5 µm or less and a surface area ratio of 15-fold or more can be formed on the stainless steel.

Fig. 4 shows the observation results of the fine crystal layer after the wet peening treatment. The fine crystal layer was formed in a depth of about 7 µm from the stainless steel surface and has a grain size of about 0.8 µm. This indicates that the fine crystal layer having a grain size of 1 µm or less and a thickness of 1 µm or more can be formed in the stainless steel surface.

### Second Embodiment

In this embodiment, a fine structure was formed on the surface of a test piece under the same conditions as those of the first embodiment except that the treatment time of the roughening etching treatment (second step) in the first embodiment was changed to 3 min. The test pieces of the second embodiment were subjected to the surficial and cross-sectional observation by SEM and the surface area evaluation. Fig. 3 shows the results of the surficial and cross-sectional observation by SEM and the surface area evaluation. It is confirmed from the surficial and cross-sectional SEM images of Fig. 3 that the fine structure having a width of 1 µm or less and a height of about 1µm is formed. The surface area of this fine structure is 15 times the area of the smooth surface. This indicates that the dimensions or surface area of the fine structure can be adjusted by varying the condition of the wet peening treatment or the etching treatment. As compared with the first embodiment, the fine structure is decreased in the surface area ratio because of the decreased height of the structure. However, even with the height of 1µm, the fine structure can achieve the 15-fold increase in the surface area ratio.

### Third Embodiment

In this embodiment, the test pieces prepared in the first embodiment were subjected to the passive film evaluation, the corrosion resistance evaluation and the adhesion evaluation. The results are described as below.

Fig. 5 shows the results of the passive film evaluation after the formation of the surface fine-structure. It is confirmed that the chromium concentration in the stainless steel surface increased by a factor of 1.5 times over the level before the formation of the surface fine-structure. This is attributable to a fact that chromium dispersed in the stainless steel remains in the stainless steel surface.

Fig. 6 shows the results of the corrosion resistance evaluation before and after the formation of the surface fine-structure. The stainless steel before the formation of the surface fine-structure had a rating number of 6 (corrosion area 0.5 to 1.0%) while the stainless steel after the formation of the surface fine-structure had a rating number of 10 (corrosion area 0.0%) . It was thus confirmed that the stainless steel was improved in the corrosion resistance by forming the surface fine-structure by the surface treatment method of the embodiment. Judging from the results of the passive film evaluation, the improved corrosion resistance is considered to be the result of the surface chromium concentration increased by the surface fine-structure forming process.

The results of the adhesion evaluation after the surface fine-structure forming process indicate no separation of the polyimide film. That is, high adhesion with the film can be achieved by applying the surface fine-structure forming process to the stainless steel.

### [Comparative Example 1]

Comparative Example 1 is described by way of an example where wet blasting treatment was used as a method for forming the surface fine-structure on the stainless steel. The test pieces were made of SUS304.

As for the conditions of the wet blasting treatment, polygonal alumina particles having a particle size of about 15µm were used as the abrasive grains under air pressure of 0.2 MPa.

The test pieces of Comparative Example 1 were subjected to the surficial and cross-sectional observation by SEM and the surface area evaluation. Fig. 3 shows the results of the surficial and cross-sectional observation by SEM and the surface area evaluation. It is confirmed from the surficial and cross-sectional SEM images of Fig. 3 that the fine structure having a width of 2 to 3 µm and a height of about 0.5 µm is formed in Comparative Example 1. The surface area of the structure of Comparative Example 1 is 3 times the area of the smooth surface.

The results of the adhesion evaluation after the surface fine-structure forming process indicate the separation of the polyimide film on the whole area.

### [Comparative Example 2]

Comparative Example 2 is described by way of an example where roughening etching treatment was used as the method for forming the surface fine-structure on the stainless steel. The test pieces were made of SUS304.

The conditions of the roughening etching treatment were the same as those of the first embodiment. The solution composition includes: 500 g/l of sulfuric acid; 90 g/l of sodium chloride; and 30 g/l of cupric chloride dehydrate. The treatment was performed at a solution temperature of 40°C for treatment time of 5 min.

The test pieces of Comparative Example 2 were subjected to the surficial and cross-sectional observation by SEM and the surface area evaluation. Fig. 3 shows the results of the surficial and cross-sectional observation by SEM and the surface area evaluation. It is confirmed from the surficial and cross-sectional SEM images of Fig. 3 that the fine structure having a width of 2 to 5 µm and a height of about 3 µm is formed in Comparative Example 2. The surface area of the structure of Comparative Example 2 is 10 times the area of the smooth surface.

The results of the adhesion evaluation after the surface fine-structure forming process indicate a partial separation of the polyimide film.

The first and second embodiments are compared with Comparative Examples 1 and 2. The surface fine-structure formed by the wet blasting treatment of Comparative Example 1 is poor in fineness, having a slightly larger distance between fine structures, which may depend upon the size of the abrasive grains. On the other hand, the surface fine-structure formed by the roughening etching treatment of Comparative Example 2 has large widths, which depend upon the size of crystal grains of the substrate because the treatment etches the crystal grain boundaries. That is, it is almost impossible for the conventional surface structure forming methods including the wet blasting treatment and the roughening etching treatment to form, on stainless steel, the surface fine-structure having a height of 5 µm or less and a surface area ratio of 15-fold or more.

### Fourth Embodiment

Next, description is made on the examples of application of the stainless steel having the surface fine-structure formed by the surface treatment method of the present invention. A preferred example of the application of the stainless steel formed with a fine irregular structure having a high surface area is an air-cooled heat exchanger performing heat exchange via gas. By applying the stainless steel subjected to the inventive surface treatment to a heat transfer part of the air-cooled heat exchanger, the heat transfer part is increased in the surface area, and heat transfer performance is improved. Because of an extremely fine irregular structure, the heat exchanger is decreased in pressure loss, thus achieving a high heat transfer accelerating effect.

In this embodiment, a shell and tube heat exchanger employing a heat transfer tube made of the stainless steel formed with the surface fine-structure by the surface treatment method of the first embodiment was evaluated for the heat transfer performance.

Fig. 7 is a structure diagram of a shell and tube heat exchanger according to a fourth embodiment of the present invention. A circular or polygonal shell 200 is provided with tube plates 202 on opposite sides thereof for supporting heat transfer tubes 201 as the heat transfer part. The tube plate 202 includes a plurality of holes arranged in a staggered fashion and penetrated by the heat transfer tubes 201. The heat transfer tubes 201 are inserted through these tube holes and secured to the tube plates 202 at opposite ends thereof. The length of the heat transfer tube 201 is equal to or more than 25 times the characteristic length D of flow. The characteristic length D of the flow along the tube group of the embodiment is defined by a hydraulic equivalent diameter. In a case where the air flow is turbulent, the heat transfer performance can be further improved by defining the length of the heat transfer tube 201 to be equal to or more than 25 times the characteristic length D of flow.

A fine structure 203 is formed on an outside surface of the heat transfer tube 201. Air 204, as a low-temperature fluid, enters the heat exchanger through a nozzle 205 disposed at a side of a lower part of the heat exchanger. The air moves up around the heat transfer tubes 201, exchanging heat with water vapor as a high-temperature fluid via heat transfer tube walls. The water vapor 206 as the high-temperature fluid enters the heat exchanger through a nozzle 207 at a top of the heat exchanger and flows through a water chamber 208 at the top of the heat exchanger and down through the heat transfer tubes 201. The water vapor 206 is condensed into compressed water by heat exchange with the air 204 as the low-temperature fluid via the heat transfer tube walls. The compressed water flows through a water chamber at a bottom of the heat exchanger so as to flow out of the heat exchanger through a nozzle at the bottom of the heat exchanger.

As a result of the application of the stainless steel formed with the surface fine-structure by the surface treatment method of the first embodiment to the heat transfer tube 201, the heat exchanger of the embodiment can be increased by about 6% in the heat transfer performance compared with that of a shell and tube heat exchanger using stainless steel subjected to no surface treatment. As described above, the application of the stainless steel formed with the surface fine-structure by the inventive surface treatment method provides for the increase in the heat transfer performance without increasing the number of heat transfer tubes. Namely, the present invention permits the reduction of the number of heat transfer tubes when achieving a desired heat transfer performance, which leads to the cost reduction of heat exchanger.

For comparison, the heat transfer tube 201 was made of the stainless steel formed with the surface fine-structure by the surface treatment method of Comparison Example 2. The resultant heat exchanger was increased by about 2.5% in the heat transfer performance compared with that of the shell and tube heat exchanger using the stainless steel subjected to no surface treatment. It was thus confirmed that the heat transfer tube 201 was improved further in the heat transfer performance as the surface area ratio thereof increased.

As for the height of the fine structure, the lower the height, the better is the fine structure as long as the surface area thereof is constant. This is because the pressure loss increases with the increase in the height of the fine structure. Although the fine structure having a height beyond a boundary layer can provide the high heat transfer accelerating effect, this effect is traded off against the increase in the pressure loss. This may result in a case where the increased pressure loss wholly cancels out the improvement in heat transfer performance. The boundary layer means a thin layer which exists in vicinity of a contact surface with gas and at which gas viscosity is non-negligible (or which is strongly affected by gas viscosity). The thickness of the boundary layer varies depending upon the specifications of the heat exchanger, namely a variety of requirements such as gas flow rate, mode of gas flow, configurations of the heat transfer part, and the like. From the standpoint of reliably reducing the pressure loss, the fine structure desirably has the lower height and the larger surface area ratio. The surface treatment method of the present invention makes it possible to form the surface fine-structure having the height of 5 µm or less and the surface area ratio of 15-fold or more, which has been impracticable for the conventional method. Therefore, the heat transfer performance higher than the conventional level can be achieved by applying the stainless steel formed with this fine structure on its surface to the heat transfer part of the heat exchanger.

As shown in Figs. 5 and 6, the stainless steel is increased in the surface chromium concentration, featuring excellent corrosion resistance. Accordingly, the stainless steel is preferably applied to the heat transfer part of the heat exchanger required of corrosion resistance.

While the fourth embodiment has been described by way of the example of the shell and tube heat exchanger, the heat exchanger to which the present invention is applicable is not limited to this. The present invention can be implemented in a heat exchanger which performs heat exchange by making contact with a gas and in which the heat transfer part making contact with the gas is made of the stainless steel. Examples of such a heat exchanger include: a fin-type heat exchanger (heat sink) for power semiconductor; a cross-fin type heat exchanger for air conditioner or automotive radiator; and the like.

### List of Reference Signs

100: STAINLESS STEEL
101: FINE CRYSTAL LAYER
102: DISPLACEMENT DEPOSITION METAL
R1: IRREGULAR STRUCTURE AFTER GRAIN REFINING TREATMENT
R2: IRREGULAR STRUCTURE AFTER ROUGHENING ETCHING TREATMENT
R3: IRREGULAR STRUCTURE AFTER DISPLACEMENT DEPOSITION METAL REMOVING TREATMENT
200: SHELL
201: HEAT TRANSFER TUBE
202: TUBE PLATE
203: FINE STRUCTURE
204: AIR
205: NOZZLE
206: WATER VAPOR
207: NOZZLE
208: WATER CHAMBER

## Claims

1. A stainless-steel (100) surface treatment method for forming a fine structure on a surface of stainless steel (100) comprising:
a first step of performing grain refining treatment for refining crystal grains in the surface of stainless steel (100); and
a second step performed, after the first step, for roughening etching the surface of stainless steel (100) with an etching solution,
**characterized in that** the roughening etching treatment of the second step is to preferentially etch grain boundaries in the surface of stainless steel (100) with a roughening etching solution which has a composition which preferably has strong acidity and contains chloride ions and transition metal ions capable of displacement deposition on iron,
and **in that** the stainless-steel (100) surface treatment method further comprises a third step, performed after the second step, for removing a displacement deposition metal (102) deposited on the surface of stainless steel (100) by the etching treatment with a solution, the composition of which does not contain chloride ions or nitrate ions that accelerate the etching of stainless steel and which has a high dissolution rate ratio for stainless steel,
wherein the grain refining treatment is any one of peening treatment, machining, and grinding and
wherein a fine crystal layer (101) formed in the surface of stainless steel (100) by the grain refining treatment of the first step has a thickness of 1 µm or more, and the crystal grains of the fine crystal layer (101) have grain sizes of 1 µm or less.

2. The stainless-steel (100) surface treatment method according to Claim 1, wherein the etching solution contains chloride ions and transition metal ions having an electric potential nobler than a standard potential of iron, and has acidity.

3. The stainless-steel (100) surface treatment method according to Claim 2, wherein the transition metal ions include any one or more of copper, silver, palladium, gold and platinum.

4. The stainless-steel (100) surface treatment method according to Claim 1, wherein in the third step, the displacement deposition metal (102) is etched away with a metal removing solution hardly dissolving stainless steel (100) and preferentially dissolving the displacement deposition metal (102), the composition of the metal removing solution preferably contains persulfate or hydrogen peroxide, if the displacement deposition metal is copper, and preferably contains potassium cyanide or ammonium peroxosulfate, if the displacement deposition metal is gold, platinum, palladium or silver.

5. The stainless-steel (100) surface treatment method according to Claim 4, wherein the displacement deposition metal (102) is copper, and the metal removing solution contains one of persulfate and hydrogen peroxide.

6. The stainless-steel (100) surface treatment method according to Claim 4, wherein the displacement deposition metal (102) is any one of silver, palladium, gold, and platinum, and the metal removing solution contains one of potassium cyanide and ammonium peroxosulfate.

7. A stainless steel material which is prepared by the stainless-steel surface treatment method according to any one of Claims 1 to 6, the stainless steel material having a fine structure portion, on its surface, which has a height of 5 µm or less and a surface area equal to or more than 15 times an area of a smooth surface, that is a surface not subjected to the process of forming the surface fine-structure.

8. A heat exchanger comprising a heat transfer part (201) for performing heat exchange by making contact with a gas (204), wherein the heat transfer part (201) making contact with the gas (204) is made of a stainless steel having a fine structure portion, on its surface, which has a height of 5 µm or less and a surface area equal to or more than 15 times an area of a smooth surface, that is a surface not subjected to the process of forming the surface fine-structure.

9. The heat exchanger according to Claim 8, wherein crystal grains in the fine structure portion (203) of the heat transfer part (201) have grain sizes of 1 µm or less.

10. The heat exchanger according to Claim 8, wherein a surface chromium concentration of the fine structure portion (203) of the heat transfer part (201) is equal to or more than 1.5 times the chromium concentration in a surface of the heat transfer part (201) which is free from the fine structure portion (203).

11. The heat exchanger according to Claim 8, wherein the surface fine-structure of the heat transfer part (201) is formed by the stainless-steel surface treatment method according to any one of Claims 1 to 6.

## Patentansprüche

1. Oberflächenbehandlungsverfahren für rostfreien Stahl (100) zum Bilden einer Feinstruktur auf einer Oberfläche aus rostfreiem Stahl (100), umfassend:
einen ersten Schritt zum Durchführen einer Kornfeinungsbehandlung zum Verfeinern von Kristallkörnern in der Oberfläche von rostfreiem Stahl (100); und
einen zweiten Schritt, der nach dem ersten Schritt zum Aufrauätzen der Oberfläche von rostfreiem Stahl (100) mit einer Ätzlösung durchgeführt wird,
**dadurch gekennzeichnet, dass** die Aufrau-Ätzbehandlung des zweiten Schrittes darin besteht, Korngrenzen in der Oberfläche von rostfreiem Stahl (100) vorzugsweise mit einer Aufrau-Ätzlösung zu ätzen, die eine Zusammensetzung aufweist, die vorzugsweise einen starken Säuregehalt aufweist und Chloridionen und Übergangsmetallionen enthält, die zur Verdrängungsabscheidung auf Eisen geeignet sind,
und dass das Oberflächenbehandlungsverfahren für rostfreien Stahl (100) ferner einen dritten Schritt umfasst, der nach dem zweiten Schritt durchgeführt wird, um ein auf der Oberfläche von rostfreiem Stahl (100) abgeschiedenes Verdrängungsabscheidungsmetall (102) durch die Ätzbehandlung mit einer Lösung zu entfernen, deren Zusammensetzung keine Chloridionen oder Nitrationen enthält, die das Ätzen von rostfreiem Stahl beschleunigen und die ein hohes Lösungsratenverhältnis für rostfreien Stahl aufweist,
wobei die Kornfeinungsbehandlung eines aus Kugelstrahlbehandlung, spanabhebender Bearbeitung und Schleifen ist, und
wobei eine feine Kristallschicht (101), die in der Oberfläche von rostfreiem Stahl (100) durch die Kornfeinungsbehandlung des ersten Schrittes gebildet ist, eine Dicke von 1 µm oder mehr aufweist, und die Kristallkörner der feinen Kristallschicht (101) Korngrößen von 1 µm oder weniger aufweisen.

2. Oberflächenbehandlungsverfahren für rostfreien Stahl (100) nach Anspruch 1, wobei die Ätzlösung Chloridionen und Übergangsmetallionen mit einem elektrischen Potential enthält, das edler ist als ein Standardpotential von Eisen, und einen Säuregehalt aufweist.

3. Oberflächenbehandlungsverfahren für rostfreien Stahl (100) nach Anspruch 2, wobei die Übergangsmetallionen eines oder mehrere von Kupfer, Silber, Palladium, Gold und Platin umfassen.

4. Oberflächenbehandlungsverfahren für rostfreien Stahl (100) nach Anspruch 1, wobei im dritten Schritt das Verdrängungsabscheidungsmetall (102) mit einer Metallentfernungslösung weggeätzt wird, die rostfreien Stahl (100) kaum löst und vorzugsweise das Verdrängungsabscheidungsmetall (102) löst, wobei die Zusammensetzung der Metallentfernungslösung vorzugsweise Persulfat oder Wasserstoffperoxid enthält, wenn das Verdrängungsabscheidungsmetall Kupfer ist, und vorzugsweise Kaliumcyanid oder Ammoniumperoxosulfat enthält, wenn das Verdrängungsabscheidungsmetall Gold, Platin, Palladium oder Silber ist.

5. Oberflächenbehandlungsverfahren für rostfreien Stahl (100) nach Anspruch 4, wobei das Verdrängungsabscheidungsmetall (102) Kupfer ist und die Metallentfernungslösung eines von Persulfat und Wasserstoffperoxid enthält.

6. Oberflächenbehandlungsverfahren für rostfreien Stahl (100) nach Anspruch 4, wobei das Verdrängungsabscheidungsmetall (102) eines von Silber, Palladium, Gold und Platin ist und die Metallentfernungslösung eines von Kaliumcyanid und Ammoniumperoxosulfat enthält.

7. Material aus rostfreiem Stahl, das durch das Oberflächenbehandlungsverfahren für rostfreien Stahl nach einem der Ansprüche 1 bis 6 hergestellt wird, wobei das Material aus rostfreiem Stahl auf seiner Oberfläche einen Feinstrukturabschnitt aufweist, der eine Höhe von 5 µm oder weniger und einen Oberflächeninhalt aufweist, der gleich oder mehr als das 15-fache eines Flächeninhalts einer glatten Oberfläche ist, d.h. eine Oberfläche, die nicht dem Prozess der Bildung der Oberflächenfeinstruktur unterzogen ist.

8. Wärmetauscher, umfassend ein Wärmeübertragungsteil (201) zum Durchführen des Wärmeaustauschs durch Kontaktnahme mit einem Gas (204), wobei das Wärmeübertragungsteil (201), das mit dem Gas (204) in Kontakt kommt, aus einem rostfreien Stahl mit einem Feinstrukturabschnitt auf seiner Oberfläche hergestellt ist, der eine Höhe von 5 µm oder weniger und einen Oberflächeninhalt aufweist, der gleich oder mehr als das 15-fache eines Flächeninhalts einer glatten Oberfläche ist, d.h. einer Oberfläche, die nicht dem Prozess der Bildung der Oberflächenfeinstruktur unterzogen ist.

9. Wärmetauscher nach Anspruch 8, wobei Kristallkörner im Feinstrukturabschnitt (203) des Wärmeübertragungsteils (201) Korngrößen von 1 µm oder weniger aufweisen.

10. Wärmetauscher nach Anspruch 8, wobei eine Oberflächenchromkonzentration des Feinstrukturabschnitts (203) des Wärmeübertragungsteils (201) gleich oder mehr als das 1,5-fache der Chromkonzentration in einer Oberfläche des Wärmeübertragungsteils (201) ist, die frei von dem Feinstrukturabschnitt (203) ist.

11. Wärmetauscher nach Anspruch 8, wobei die Oberflächenfeinstruktur des Wärmeübertragungsteils (201) durch das Oberflächenbehandlungsverfahren für rostfreien Stahl nach einem der Ansprüche 1 bis 6 gebildet wird.

## Revendications

1. Procédé de traitement de surface d'acier inoxydable (100) pour former une fine structure sur une surface d'acier inoxydable (100) comprenant :
une première étape consistant à exécuter un traitement d'affinage de grains pour affiner les grains de cristaux dans la surface de l'acier inoxydable (100) ; et
une seconde étape, exécutée après la première étape, pour rendre rugueuse par attaque chimique la surface d'acier inoxydable (100) avec une solution d'attaque,
**caractérisé en ce que** le traitement d'attaque afin de rendre la surface rugueuse de la seconde étape est destiné à attaquer préférentiellement les frontières de grains dans la surface de l'acier inoxydable (100) avec une solution d'attaque afin de rendre la surface rugueuse qui a une composition présentant de préférence une forte acidité et contenant des ions chlorure et des ions de métal de transition capable de déposition par déplacement sur du fer,
et **en ce que** le procédé de traitement de surface d'acier inoxydable (100) comprend de préférence une troisième étape, exécutée après la seconde étape, pour supprimer un métal de déposition par déplacement (102) déposé sur la surface de l'acier inoxydable (100) par le traitement d'attaque avec une solution, dont la composition ne contient pas d'ions chlorure ou d'ions nitrate qui accélèrent l'attaque de l'acier inoxydable et qui présente un taux de dissolution élevé pour l'acier inoxydable,
dans lequel le traitement d'affinage de grains est un traitement quelconque parmi un traitement de grenaillage, un traitement d'usinage, et un traitement par meulage, et
dans lequel une fine couche de cristal (101) formée dans la surface de l'acier inoxydable (100) par le traitement d'affinage de grains de la première étape a une épaisseur de 1 µm ou plus, et les grains de cristaux de la fine couche de cristal (101) ont des tailles de grains de 1 µm ou moins.

2. Procédé de traitement de surface d'acier inoxydable (100) selon la revendication 1, dans lequel la solution d'attaque contient des ions chlorure et des ions de métal de transition ayant un potentiel électrique plus noble qu'un potentiel standard du fer, et présente une acidité.

3. Procédé de traitement de surface d'acier inoxydable (100) selon la revendication 2, dans lequel les ions de métal de transition incluent un quelconque ou plusieurs des ions suivants : cuivre, argent, palladium, or et platine.

4. Procédé de traitement de surface d'acier inoxydable (100) selon la revendication 1, dans lequel, dans la troisième étape, le métal de déposition par déplacement (102) est supprimé par attaque avec une solution de suppression de métal qui dissout à peine l'acier inoxydable (100) et qui dissout préférentiellement le métal de déposition par déplacement (102), la composition de la solution de suppression de métal contenant de préférence du persulfate ou du peroxyde d'hydrogène, si le métal de déposition par déplacement est du cuivre, et contient de préférence du cyanure de potassium ou du peroxosulfate d'ammonium, si le métal de déposition par déplacement est de l'or, platine, palladium ou argent.

5. Procédé de traitement de surface d'acier inoxydable (100) selon la revendication 4, dans lequel le métal de déposition par déplacement (102) est du cuivre, et la solution de suppression de métal contient soit du persulfate soit du peroxyde d'hydrogène.

6. Procédé de traitement de surface d'acier inoxydable (100) selon la revendication 4, dans lequel le métal de déposition par déplacement (102) est un métal quelconque parmi argent, palladium, or et platine, et la solution de suppression de métal contient soit du cyanure de potassium soit du peroxosulfate d'ammonium.

7. Matériau en acier inoxydable qui est préparé par le procédé de traitement de surface d'acier inoxydable selon l'une quelconque des revendications à 6, le matériau en acier inoxydable ayant une portion à fine structure sur sa surface, qui a une hauteur de 5 µm ou moins et une superficie égale ou supérieure à 15 fois une superficie d'une surface lisse, c'est-à-dire une surface qui n'est pas soumise au processus de formation de surface à fine structure.

8. Échangeur de chaleur comprenant une partie de transfert de chaleur (201) pour effectuer un échange de chaleur en établissant un contact avec un gaz (204), dans lequel la partie de transfert de chaleur (201) qui établit un contact avec le gaz (204) est faite d'un acier inoxydable ayant une portion à fine structure, sur sa surface, qui a une hauteur de 5 µm ou moins et une superficie égale ou supérieure à 15 fois une superficie d'une surface lisse, c'est-à-dire une surface qui n'est pas soumise au processus de formation de surface à fine structure.

9. Échangeur de chaleur selon la revendication 8, dans lequel les grains de cristaux dans la portion à fine structure (203) de la partie de transfert de chaleur (201) ont des tailles de grains de 1 µm ou moins.

10. Échangeur de chaleur selon la revendication 8, dans lequel une concentration de chrome en surface de la portion à fine structure (203) de la partie de transfert de chaleur (201) est égale ou supérieure à 1,5 fois la concentration de chrome dans une surface de la partie de transfert de chaleur (201) qui est dépourvue de la portion à fine structure (203).

11. Échangeur de chaleur selon la revendication 8, dans lequel la surface à fine structure de la partie de transfert de chaleur (201) est formée par le procédé de traitement de surface d'acier inoxydable selon l'une quelconque des revendications 1 à 6.
